

## UNITED STATES PATENT OFFICE

1,929,955

## LUBRICANT

Roy F. Nelson, Port Arthur, Tex., assignor to The Texas Company, New York, N. Y., a corporation of Delaware

No Drawing. Application December 13, 1930  
Serial No. 502,256

12 Claims. (Cl. 87—c)

This invention relates to lubricants, and more particularly to cutting oils used for drilling, thread cutting and similar lathe machine work.

The use of cutting oils in ordinary operations of machine shops is well known. The function of the cutting fluid is usually two-fold; that is, as a cooling agent to keep the drilling or cutting tools from over-heating, and as a lubricant to alleviate friction between the contacting parts.

10 The requirement of a good cutting fluid is, therefore, that it provide a certain degree of cooling, and especially that it have sufficient oiliness to adhere to the working parts and reduce the friction to a minimum. Sometimes it is necessary to cool the working parts with water or similar fluid having a high specific heat. In the latter practice, it is desirable that the lubricant will not wash from the metal surfaces and often preferable that it form an emulsion with the cooling

15 agent. Straight mineral oils, are ordinarily good lubricants, but they are not entirely satisfactory as cutting oils. Other sources have, accordingly, been sought, or the mineral oils have been treated to transform them into satisfactory lubricants

20 for this purpose.

Various methods of treating mineral oils to produce satisfactory cutting oils have been employed heretofore. Certain animal oils, such as lard oil, because of their oiliness have been 30 blended with mineral oil to confer greater efficiency on the lubricant. The quantity of lard oil required is usually quite large, thereby making the cutting oil somewhat expensive. Emulsifying agents such as soaps have sometimes been 35 added to mineral oil to produce a cutting oil which will have increased oiliness, and more especially to confer on the oil the property of emulsifying with the cooling fluid which may be added. In this way, instead of the oil entirely washing away

40 when a cooling agent is applied, an emulsion is formed which contains sufficient oil to provide a certain degree of lubrication. Sulphurized oils comprising vegetable oils or mineral oils, with limited quantities of sulphur incorporated there-

45 in, have also been used to advantage to increase the viscosity, oiliness and emulsifying properties of cutting oils. The efficiency of the latter type of oils has very largely depended on the sulphur content, which has been somewhat limited due

50 to the low solubility of sulphur in the oil and the inability to incorporate large quantities therein.

The present invention has to do with an improved sulphurized mineral cutting oil prepared in a novel manner and having a particularly high sulphur content. Cutting oils comprising miner-

al oil, sulphur and a sulphur solvent are old in the art and no claim is made, broadly, to such a product, but, as far as I am aware, no cutting oil containing the high percentage of sulphur of my product has been successfully prepared prior to 60 the invention. Furthermore, incorporation of sulphur into mineral oils to prepare cutting oils is recognized as old in the art, but all the prior methods, to the best of my knowledge, have involved treating the oil in the presence of free 65 sulphur, at various temperatures, under atmospheric pressure. One of the important features of my process that is considered novel and which has produced unexpected results, resides in the incorporation of the sulphur into the oil under 70 substantial superatmospheric pressure.

More particularly, according to the invention, a mineral oil, preferably having a viscosity of at least or exceeding 70 seconds Saybolt at 100° F., is mixed with sulphur and the mixture heated 75 under pressure to a temperature in excess of 300° F., preferably 350° F. to 450° F. The pressure may be applied from an extraneous source, but it is usually more convenient to allow the mixture to build up a self-generated pressure by the evolution of reaction gases, such as hydrogen sulphide. A pressure of about 75 to 150 lbs. per sq. in. is preferable, although best results have been obtained with a pressure of approximately 100 80 lbs. per sq. in. The amount of sulphur retained 85 by the oil has been found to increase with the time the mixture is digested or held under the operating conditions of temperature and pressure. The time varies somewhat with the character of the oil, and the degree of sulphurization 90 desired; however, a period of 2 to 10 hours has been found satisfactory in most instances. The viscosity of the oil is usually increased considerably by the incorporation of sulphur therein. This increase may range from 25 to 100 seconds 95 Saybolt or more. It is preferable that the finished product have a viscosity in excess of 75 seconds Saybolt at 100° F.

The reaction between the sulphur and oil has been found to liberate large quantities of reaction gases, such as hydrogen sulphide, which normally escape but under pressure either combine with or remain dissolved in the oil after the pressure is released. The latter is particularly true when the reaction period provides insufficient time for complete absorption of the sulphur by the oil. The hydrogen sulphide imparts a disagreeable odor if allowed to remain in the finished product. It is preferable, therefore, to remove the dissolved gases as completely 110

as possible. This may be done by applying a vacuum to the oil to draw out the dissolved gases or to blow a stream of gas, such as air, through the oil to carry out the hydrogen sulphide. It 5 may be desirable in some cases to mix substances with the mineral oil and sulphur mixture, which will absorb or destroy any foul gases. Sulphur dioxide has been suggested for this purpose. Furthermore, it may sometimes be advantageous 10 to add materials which not only are capable of absorbing sulphur and destroying the foul odor of the sulphur containing gases, but also will give a positive and more pleasant odor to the finished product. Pine tar has been used with this object 15 in view.

Oils prepared in accordance with the invention are characterized by their high sulphur content. For example, a pale oil with the viscosity of about 20 77 seconds Saybolt at 100° F. heated with sulphur for 10 hours at about 390° F. and under a pressure of approximately 100 lbs. per sq. in., produced a finished oil containing 6.87% sulphur and a viscosity of 136 seconds Saybolt at 100° F. A light paraffin distillate with a viscosity of 25 86 seconds Saybolt at 100° F., treated by substantially the same procedure, produced a cutting oil having 8.6% sulphur and a viscosity of 106 seconds Saybolt at 100° F. Other products containing sulphur in quantities ranging from 30 4% to 10% may be easily prepared. From 2% to 10% sulphur absorbing material, such as pine tar, may be added to the above product if desired.

Obviously many modifications and variations of the invention, as hereinbefore set forth, may 35 be made without departing from the spirit and scope thereof, and therefore only such limitations should be imposed as are indicated in the appended claims.

I claim:

- 40 1. The method of treating mineral oils to produce cutting fluids, which comprises mixing sulphur with an oil having a viscosity of at least 70 seconds Saybolt at 100° F. and heating the mixture to a temperature at which reaction between 45 the oil and sulphur occurs while maintaining the reacting materials under a superatmospheric pressure of about 75 lbs. to 150 lbs. per sq. in.
2. A process substantially as described in claim 1 in which the superatmospheric pressure is self-generated by confining vapors and gases evolved during the heating operation.
3. A process substantially as described in claim 1 in which the temperature is 350° F. to 450° F.

55

60

65

70

75

4. The method of treating mineral oils to produce cutting fluids, which comprises heating a mixture of mineral oil and sulphur to a temperature of about 400° F. and at a pressure of about 100 lbs. per sq. in. for a period of time sufficient to incorporate in said oil a substantial amount of sulphur. 80

5. A method substantially as described in claim 4 in which the time under pressure is 2 to 10 hours. 85

6. The method substantially as described in claim 4 in which the amount of sulphur incorporated is 4% to 10% of the weight of the oil. 90

7. The method of preparing sulfur cutting oils which comprises digesting a viscous hydrocarbon oil in the presence of free sulfur at a temperature in excess of 300° F. and under a superatmospheric pressure of about 75 lbs. to 150 lbs. per sq. in. 95

8. In the preparation of sulfurized cutting oils wherein sulfur is incorporated in an oil of viscosity of at least 70 seconds Saybolt at 100° F. under the influence of heat, the improvement which comprises maintaining a superatmospheric pressure of at least 75 lbs. per sq. in. on the oil during the sulfurizing operation. 100

9. The method which comprises incorporating 100 sulphur into a lubricating oil while maintaining the oil at an elevated temperature and under a pressure in excess of 75 lbs. per sq. in. 105

10. The method of sulfurizing oils which comprises subjecting a hydrocarbon oil having a viscosity of at least 70 seconds Saybolt at 100° F. to the action of sulfur at a temperature in excess of 300° F. and under a superatmospheric pressure of at least 75 lbs. per sq. in. 110

11. In the manufacture of sulfurized oils 110 wherein sulfur is incorporated into a hydrocarbon oil while maintaining the oil under substantial superatmospheric pressure and at a temperature sufficiently high to effect reaction between the sulfur and the oil, the step of removing gases, of 115 disagreeable odor, which are liberated and would partially remain in the finished oil after release of the pressure, by blowing the finished oil with a stream of gas to carry out the undesirable gases. 120

12. A mineral oil product consisting essentially 120 of a paraffinic lubricating oil of at least 70 seconds Saybolt viscosity at 100° F. containing about 4% to 10% by weight of sulfur and resulting from the heating of the oil with sulfur under substantial superatmospheric pressure. 125

ROY F. NELSON.

130

135

140

145

150